

## UNITED STATES PATENT OFFICE.

LESTER KIRSCHBRAUN, OF CHICAGO, ILLINOIS.

## PROCESS OF MAKING WATERPROOF COMPOSITION AND PRODUCT PRODUCED THEREBY.

No Drawing. Application filed October 20, 1920, Serial No. 418,316. Renewed October 8, 1926.

This invention relates to improvements in the production of a waterproof paper, a felted web in which a normally adhesive waterproofing agent, such as asphalt, is incorporated in the paper simultaneously with the web-forming operation. Among its salient objects are to provide a process whereby the asphalt or other bituminous or hydrocarbon material of a normally adhesive character is made temporarily non-adhesive; to provide a process whereby this transformation to a non-adhesive state is accomplished by a process of dispersion into water by means of an emulsifying agent, a process whereby waterproof compositions, such as paper, fabrics, felts, and the like, similar to those used in the manufacture of prepared roofings, may be made with the waterproofing substances intimately incorporated in the stock of the composition instead of being saturated or coated as is the usual practice; to provide a process whereby the finely dispersed particles of asphalt, tar, pitches of vegetable, animal or mineral origin, resins or resinous materials to be incorporated with the fibre, felt or paper stock are emulsified with a water and an emulsifying agent so that each particle of the adhesive substance is surrounded by non-adhesive films, which are subsequently removed after the web has been dried at which time the waterproofing substance assumes its normal adhesive state; to provide a process in which relatively high melting point asphalt, such as oxidized asphalt, may be temporarily modified to a low melting point and subsequently returned to substantially its original state; to provide a process in which the bituminous material undergoing emulsification is superficially reacted upon to produce a non-adhesive protective film, and to provide a process in which the bituminous material is converted to a form in which it can be readily precipitated upon the fibres.

This process resides in the conversion of asphalt, or other bituminous or hydrocarbon materials, which are normally adhesive in nature, to a finely divided non-adhesive form and in incorporating the same with paper stock, felt or fibrous material in the making of waterproof composition. This

asphalt may be either native, pure or containing mineral matter softened, if desired, by means of fluxing oils or it may be the product of distillation or oxidation of asphaltic petroleums. These asphalts, or other hydrocarbon substances are incorporated into the body of the felt or fibrous stock by emulsifying them with a combination of clay and water and mixing the emulsion with the stock to form an emulsion having the adhesive material in the internal phase and a water in the external phase.

Heretofore, asphalts have been combined with paper stock and felted or fibrous material by grinding the mineral asphalt or hydrocarbon materials and combining them while in a solid state. The product from this combination is not altogether satisfactory as the asphalt does not incorporate itself with the fibrous materials nor does it coalesce to the extent the asphalt does when combined in an emulsified form.

It is essential in making this emulsion that sufficient water is added to keep the emulsion in the proper form, that is, it is necessary that the water be in the external phase and the adhesive or asphaltic material in the internal phase. This is important, due to the fact that when the emulsion is combined with the paper stock or fibrous material and is run over a paper machine the substance will not adhere to the screens and blankets of the paper forming machine.

In order to produce the emulsion referred to I use clay, containing a large proportion of colloidal material as the emulsifying agent, but obviously other finely divided powders, which produce an emulsion of a non-adhesive character, may be used.

The process may be run as a batch or continuous process and success may be obtained with either type, if the proportions of the ingredients used are carefully added.

More specifically, in the making of this emulsion I flux asphalt by heating with oleic acid and thoroughly mix them together. The most advantageous temperature for this combination depends primarily upon the melting point of the asphalt. This combination, while molten, is then emulsified with clay in colloidal form, held in suspension in a water vehicle. A thorough emulsification

may be obtained by violent agitation of the two during the mixture.

After these materials have been thoroughly emulsified, the emulsion is added to any suitable fibrous stock, such as that put over a paper machine. This stock may consist of rags, papers, or other fibrous stock. The fibrous stock and emulsion are then mixed in beaters until the emulsion is thoroughly incorporated throughout the fibres. To this mixture is then added a solution of lime or analogous agent, such as alum, which will react to form insoluble and precipitable oleates. The addition of the oleic acid to the initial mixture permits the use of higher melting point asphalt in the emulsification and produces superficial reaction resulting in films, which are formed about the particles of asphalt. These films are more resistant than a water film and, therefore, add to the non-adhesive character of the emulsion.

After the asphalt emulsion has been thoroughly mixed in the fibrous stock, the addition of the solution of lime, or analogous agent with an alkali tends to coagulate the particles of asphalt upon the individual fibres, producing a very uniform waterproofing composition when run over a paper forming machine, and dried. The paper forming machine referred to may be of the Fourdrinier or cylinder type machine, the web being formed in either case by means of a screen either running continuously over a series of rolls or mounted upon a single roll and caused to adhere thereto and pass therefrom by contacting couch rolls.

The character of the asphalt and the degree of incorporation may be varied according to the desired form of waterproofing material and the amount of the waterproofing substances used. The emulsification of the asphalt and oleic acid mixture with the clay is preferably done at a temperature substantially at or above the melting point of the asphaltic mixture.

As the paper stock with the emulsion thoroughly incorporated therein is run over a paper machine, a greater part of the water is drawn therefrom, the sheet passed over driers when the asphalt or other waterproofing substance will re-assume its adhesive nature and intimately coalesce with the fibrous stock, and flow through the sheet thus producing a very uniform product.

I claim as my invention:

1. A process for making a felted fibrous composition comprising fluxing a waterproofing substance with a fatty acid dispersing same in an aqueous medium by means of an emulsifying agent, mixing the emulsion with a fibrous pulp contained in an aqueous vehicle, adding a reagent to produce an insoluble soap upon the surface of the particles of waterproofing substance and passing

the mixture over a paper-forming machine to form a sheet-like web.

2. A process for making a felted fibrous composition having a waterproofing binder comprising fluxing a heated asphaltic waterproofing substance with an asphalt soluble acid and emulsifying the mixture with finely divided colloidal powders held in suspension in an aqueous vehicle, mixing the emulsion with a fibrous pulp in an aqueous vehicle and adding a reagent to produce an insoluble soap with an asphalt-soluble acid before finally passing the composition over the paper machine.

3. A process for making a felted waterproof fibrous sheet having a waterproof binder incorporated therein, comprising forming an emulsion, in which the binder is fluxed with a fatty acid and the mixture finely dispersed through colloidal clayey particles held in suspension in an aqueous vehicle with the adhesive binder in the internal and the water in the continuous phase, mixing the emulsion with the fibrous pulp and adding a reagent to produce an insoluble soap with the fatty acid before finally felting the fibrous pulp and removing the water by passing the mixture over a paper-making machine.

4. A process for making a felted fibrous sheet having a waterproof bituminous binder incorporated therein, comprising fluxing the binder with a fatty acid and emulsifying the mixture with colloidal clayey particles in an aqueous vehicle to produce the finely dispersed binder substance in the internal phase and an aqueous film constituting the continuous phase, thoroughly incorporating the emulsion with a fibrous pulp in an aqueous vehicle, and causing the emulsion to precipitate on the fibrous particles by adding a precipitating agent.

5. A process for making a felted fibrous sheet having a waterproof bituminous binder incorporated therein, comprising fluxing the binder with a fatty acid to reduce the melting point of the binder and emulsifying the mixture with colloidal clayey particles in an aqueous vehicle to produce the finely dispersed binder substance in the internal phase and an aqueous film constituting the continuous phase, thoroughly incorporating the emulsion with a fibrous pulp in an aqueous vehicle and causing the emulsion to precipitate on the fibrous particles by the addition of a precipitating agent and finally passing the composition over a paper machine.

6. A process of making felted fibrous compositions, which comprises fluxing a waterproofing substance with a fatty acid and introducing an agent to emulsify the mixture, mixing the emulsion thus formed with fibrous pulp contained in an aqueous vehicle, and adding a reagent to produce an insoluble

ble soap upon the surface of the particles of waterproofing substance, and sheeting the mixture on a paper machine.

7. The process of making a felted fibrous composition, which comprises fluxing a relatively high melting point asphalt with an asphalt-soluble acid to thereby lower its melting point, and mixing an agent therewith

to form an emulsion, mixing the emulsion thus formed with fibrous pulp contained in an aqueous vehicle, and adding a re-agent to produce an insoluble soap upon the particles of asphalt, and sheeting the mixture on a paper machine. 10

LESTER KIRSCHBRAUN.